

## 1

2,694,688

## ANTISTATIC COMPOSITIONS FOR TEXTILES

Lehman E. Hughes, New Castle, Del., assignor to E. I. du Pont de Nemours and Company, Wilmington, Del., a corporation of Delaware

No Drawing. Application February 27, 1953,  
Serial No. 339,454

3 Claims. (Cl. 260—29.6)

This invention relates to certain polymeric alkyl sulfate quaternary ammonium salts of the acrylyloxyethylamine type and to the treatment of textiles therewith.

One disadvantage of textile fibers and particularly of fabrics prepared from synthetic hydrophobic materials, and of all textile fibers treated with conventional resin finishes, is that they tend to develop a static electrical charge. This charge is objectionable during the manufacture of the textile and in the finished garment. During manufacture the static charge on the fibers or fabric interferes with their convenient handling during spinning, reeling, weaving and the like. Finished articles which are designed to drape like cotton or wool articles fail to do so properly due to their electrostatic charge and often cling uncomfortably to the wearer. Furthermore, such textiles tend to collect dust and lint, and the electric discharge itself is bothersome.

Many treating agents have been proposed to impart anti-static effects to textiles of this type. However, none of the proposed agents is entirely satisfactory, either because of their effectiveness or their resistance to washing and dry cleaning. Many of these anti-static agents are effectively transferred to the textile materials only with great difficulty.

It is therefore an object of this invention to provide an effective anti-static composition which is highly resistant to washing and dry cleaning. Another object is the provision of an anti-static agent which imparts a durable anti-static effect to synthetic textile fibers and fabrics. Another object is the provision of agents which may be applied by simplified treatments to the textiles rendering them substantially permanently anti-static. Other objects will appear as the description of the invention proceeds.

These and other objects are accomplished by a composition in the form of an aqueous dispersion which comprises, in proportion, about 15 parts by weight of a water-soluble polymer of a quaternary salt of an acrylyloxy-alkyltrialkylamine in which each alkyl group has from 1 to 4 carbon atoms; about 2 to 10 parts by weight of a water-soluble salt of an aliphatic alcohol sulfate having from 8 to 20 carbon atoms; about 5 to 10 parts by weight of one or more saturated aliphatic monohydric alcohols having from 2 to 12 carbon atoms, but averaging on a weight basis of from 3.0 to 5.0 carbon atoms; about 2.0 to 20 parts by weight of a mixture of monocyclic terpene hydrocarbons; and the balance being water to give 100 parts by weight.

The term "water-soluble" is used to mean that the salt is soluble in water. Those of the present invention are soluble at least to the extent of about 5% by weight, at about 70° to 80° C. although the solution may be colloidal rather than a true solution. At any rate, the solution should be homogeneous and capable of dilution at the working concentration. The average of carbon atoms in the alcohol containing from 2 to 12 carbon atoms on a weight basis is obtained by adding the product of the number of carbon atoms in each alcohol by the weight percent used of the alcohol, and dividing the sum by 100.

The agents are applied to textiles by any suitable procedure which leaves on the article treated about 0.05% to about 2% or even higher under extreme conditions of the active ingredient. The preferred range is usually from 0.25% to 0.9% of the methylsulfate salt, or the proportionately higher equivalent of the reacted salt

## 2

based on the dry weight of the textile or other material treated.

While many of the quaternary compounds defined above impart satisfactory anti-static properties to textiles, it has been found that the polymer of beta-methacrylyloxyethylmethyldiethyl ammonium methylsulfate, together with sodium hexadecenyl sulfate in the above combination yields exceptionally satisfactory results.

The monocyclic terpene hydrocarbons present in the preferred dispersions are the unsaturated monocyclic hydrocarbons derived from turpentine. These are readily available on the open market in several grades and contain dipentene, terpinolene and terpinene as their primary constituents.

15 The dispersions are prepared conveniently by adding an aqueous solution of the long-chain alkyl sulfate, plus the alcohols and terpenes, to an aqueous solution of the quaternary ammonium salt at room temperature. A reaction takes place between the quaternary ammonium salt and the long-chain alkyl sulfate. Some of the short-chain alkyl sulfate anions are replaced by long-chain alkyl sulfate anions, throwing out some of the quaternary compound from solution in most instances. The resulting product is, therefore, actually a dispersion of 20 this solid in the liquid components and is made homogeneous with a fine particle size by stirring vigorously at about 25 room temperature during the reaction.

These dispersions may be applied to the fabric by a padding procedure, and if desired, may be applied in 30 conjunction with any of the ordinary crease-resistant resin finishes for textiles as will be apparent from certain of the following examples. Among the resins used for this purpose are the methylol ureas, methylol melamines, their ethers and 1,3-bis(hydroxymethyl)-35 imidazolidone. These agents impart stiffness, crease-resistance, dimensional stability and other properties to textiles.

It has been found that ordinary loadings of these resins and finishes usually increase the static properties of textiles, and that the compositions of the present invention solve this particular problem very effectively.

The following examples are given by way of illustration, but it is to be understood that any of the quaternary ammonium compounds and water-soluble, long-chain sulfates falling within the above generic description of the invention may be substituted for any of those given in the examples with comparable results.

The agents of this invention are applied to textiles and tested as described in Examples I and II of copending 50 application Serial No. 260,119, filed December 5, 1951.

*Example I*

18.4 parts of sodium hexadecenyl sulfate (25% to 30% aqueous paste); 6.15 parts of mixed monocyclic 55 terpene hydrocarbons; 4.9 parts of 95% ethyl or isopropyl alcohol; and 3.05 parts of C<sub>8</sub> alcohol (primarily n-octanol) are mixed to yield a clear, light yellow fluid. This solution is added slowly with agitation to a mixture of 50 parts of a 30% aqueous solution of poly-beta-methacrylyloxyethylmethyldiethylmethyl ammonium methylsulfate and 17.5 parts of water. A viscous, pourable white dispersion is formed which is stable at any dilution with water. When diluted to 1% (based on the polymer content) and padded onto nylon, polyacrylonitrile and polyethylene terephthalate fabrics, the anti-static action is excellent when measured as described above. This effect remains very good after repeated hot aqueous rinsing and after soap scouring.

*Example II*

70 Example I is repeated using 25 parts of sodium hexadecenyl sulfate (25% to 30% aqueous paste); 7.5 parts of mixed monocyclic terpene hydrocarbons; 3 parts of 95% ethyl alcohol; 3.5 grams of C<sub>8</sub> alcohol (primarily n-hexanol); 50 parts of a 30% aqueous solution of poly-beta-methacrylyloxyethylmethyldiethylmethyl ammonium methylsulfate; and 11 parts of water. A similar product is produced which has comparable properties as an anti-static agent.

*Example III*

80 Example I is repeated using 32.5 parts of sodium hexa-

decenyl sulfate (25% to 30% aqueous paste); 10.0 parts of mixed monocyclic terpene hydrocarbons; 3 parts of 95% ethyl alcohol; 3 parts of n-amyl alcohol; 50 parts of a 30% aqueous solution of poly-beta-methacrylyoxyethylidethylmethyl ammonium methylsulfate; and 1.5 parts of water. The product is a stable dispersion as is, and also when diluted with water to about 1%.

*Example IV*

Example I is repeated using 15 parts of sodium hexadecenyl sulfate (25% to 30% aqueous paste); 4 parts of 95% ethyl alcohol; 2.5 parts of C<sub>8</sub> alcohol; 50 parts of a 30% aqueous solution of poly-beta-methacrylyoxyethylidethylmethyl ammonium methylsulfate; and 28.5 parts of water. When this product is diluted with water to 1%, the stability of the dispersion is not as good as in the preceding examples.

*Example V*

Similar high anti-static properties of good durability are developed when Example I is repeated using poly-beta-methacrylyoxyethyltrimethyl ammonium methylsulfate. Likewise, when poly-beta-methacrylyoxyethyltriethyl ammonium ethylsulfate is substituted for the quaternary ammonium compound of Example I, the resulting dispersion is suitable for imparting good anti-static protection to textiles made of acetate, nylon, polyacrylonitrile and polyethylene terephthalate.

*Example VI*

Substitution of each of the following for sodium hexadecenyl sulfate in Example I gives a dispersion suitable for imparting attractive anti-static properties to the above-mentioned hydrophobic fibers:

Sodium octyl sulfate  
 Sodium dodecyl sulfate  
 Potassium dodecyl sulfate  
 N-diethylcyclohexyl ammonium dodecyl sulfate  
 Sodium salt of mixed dodecyl-tetradecyl sulfate (from technical dodecyl alcohol)  
 Sodium salt of the sulfates of mixed dodecyl-tetradecyl alcohols condensed with about one mol of ethylene oxide.  
 Ammonium dodecyl sulfate  
 Sodium octadecenyl (oleyl) sulfate  
 Sodium salt of the sulfate of octadecenyl alcohol, condensed with about one mol of ethylene oxide  
 Sodium salt of mixed C<sub>10</sub>-C<sub>20</sub> alkenyl sulfates (alcohols derived from sodium reduction of sperm oil)

*Example VII*

A dispersion is prepared by mixing 20 parts of poly-beta-methacrylyoxyethylidethylmethyl ammonium methylsulfate with 20 parts of a solution of 3.1 parts of sodium hexadecenyl sulfate; 11.6 parts of a monocyclic terpene (by-product of camphor manufactured from turpentine); 2.7 parts of ethyl alcohol; 1.8 parts of technical octyl alcohol; 0.8 part of decyl alcohol; 1.1 parts of isopropyl alcohol; and 12.8 parts of water. The dispersion is applied to fabrics composed of nylon, polyacrylonitrile, polyethylene terephthalate and of cellulose acetate by padding in such a way that 0.3% by weight of active ingredient was obtained on each of the fabrics. The anti-static properties measured at relative humidities from 20% to 75% as described above were all good to excellent.

A similar good dispersion results from reducing the amount of complex dispersing agent to 10 parts.

In every case, both with and without the anti-static agent, the pieces of textile have a pleasing hand and satisfactory degrees of crease-resistance and dimensional stability.

The present invention is particularly useful in reducing the anti-static properties of textile materials including fibers, yarns, threads and fabrics prepared from synthetic materials having high electrical resistance, such as those prepared from cellulose acetate, nylon, polyacrylonitrile, and polyethylene terephthalate. Another advantage of the present invention is that the anti-static agents may be applied simultaneously with resinous, crease-resistant materials which normally increase the static effects of the textiles so treated, but when these resins are applied with the compositions of the present invention the static effects of the resin are obviated. This invention also provides a direct route to an anti-static finish which is not slimy in the presence of water.

It will be apparent that many widely different embodiments of the invention may be made without departing from the spirit and scope thereof, and therefore it is not intended to be limited except as indicated in the appended claims.

I claim:

1. An aqueous dispersion for imparting anti-static properties to materials which tend to accumulate an electro-static charge which comprises, in proportion, about 15 parts by weight of a water-soluble polymer of a quaternary salt of an acrylyoxyalkyltrialkylamine in which each alkyl group has from 1 to 4 carbon atoms; about 2 to 10 parts by weight of a water-soluble salt of an aliphatic alcohol sulfate having from 8 to 20 carbon atoms; about 5 to 10 parts by weight of one or more saturated, aliphatic alcohols having from 2 to 12 carbon atoms, but averaging, on a weight basis, within the range of 3.0 to 5.0 carbon atoms; about 2.0 to 20 parts by weight of a mixture of monocyclic terpene hydrocarbons; the balance of the composition being water to give a total of 100 parts by weight.

2. The composition of claim 1 having the approximate following composition in parts by weight:

|                                                             |      |
|-------------------------------------------------------------|------|
| Polymeric quaternary compound                               | 15.0 |
| Sodium salt of an alkyl sulfate having 8 to 20 carbon atoms | 4.5  |
| Ethyl alcohol                                               | 5.0  |
| An alcohol having 8 carbon atoms                            | 3.0  |
| Monocyclic terpene hydrocarbon mixture                      | 6.5  |
| Water to make 100 parts.                                    |      |

3. The composition of claim 1 having the approximate following composition in parts by weight:

|                                                                         |      |
|-------------------------------------------------------------------------|------|
| Polymeric beta - methacrylyoxyethylidethylmethyl ammonium methylsulfate | 15.0 |
| Sodium salt of octadecenyl sulfate                                      | 4.5  |
| Ethyl alcohol                                                           | 5.0  |
| An alcohol having 8 carbon atoms                                        | 3.0  |
| Monocyclic terpene hydrocarbon mixture                                  | 6.5  |
| Water to make 100 parts.                                                |      |

References Cited in the file of this patent

UNITED STATES PATENTS

|           |        |               |
|-----------|--------|---------------|
| Number    | Name   | Date          |
| 2,626,786 | Carnes | Jan. 27, 1953 |